

Sept. 19, 1967

F. TOMHOLT ET AL

3,341,940

METHOD OF MAKING A PERMANENT MAGNET

Filed March 28, 1963



INVENTORS  
FRITS TOMHOLT  
BY WILLEM EISE WITTEVEEN

*Frank R. Jiglar*  
AGENT

3,341,940

**METHOD OF MAKING A PERMANENT MAGNET**  
Frits Tomholt and Willem Eise Witteveen, Emmasingel,  
Eindhoven, Netherlands, assignors to North American  
Philips Company, Inc., New York, N.Y., a corporation  
of Delaware

Filed Mar. 28, 1963, Ser. No. 268,782  
Claims priority, application Netherlands, Mar. 29, 1962,  
276,592

4 Claims. (Cl. 29—608)

**ABSTRACT OF THE DISCLOSURE**

A method and apparatus for manufacture of permanent anisotropic magnets, particularly ceramic permanent magnets, in which a permanent magnet material is finely-divided, placed in a hermetically sealed receptacle, the material whirled to form a dust cloud from which particles are separated by a magnetic field which form conglomerates. These conglomerates are then removed from the receptacle, compacted into a body in the presence of a magnetic field and sintered to form a coherent body which is a permanent magnet.

Our invention relates to a method of manufacturing a magnetically anisotropic body and to a magnetically anisotropic body manufactured by this method.

Magnetically anisotropic magnets have been made by compressing a finely divided permanent magnetic material in a magnetic field which orients the magnetic material, after which the compressed oriented material is sintered into a highly coherent body. Naturally, it is desirable in this case that the magnetic orientation produces a maximum effect, so that the compressed mass is indeed strongly magnetically anisotropic. However, it has been found that the particles which should be oriented mutually in parallel with their easy direction of magnetization show a tendency to conglomerate because they attract each other magnetically while forming magnetically isotropic conglomerates, as a result of which the effect of the magnetic orientation is decreased.

It is a principal object of our invention to minimize the tendency of the particles to form isotropic conglomerates during orientation.

A further object of our invention is to provide a method of manufacturing anisotropically permanent magnets having improved anisotropic properties. These and further objects of the invention will appear as the specification progresses.

According to the invention, we completely disintegrate the material from which a permanent magnet is to be made, in a closed receptacle, to a powder having an average particle size under 1 micron. This powder is then whirled or centrifuged to form a cloud of dust from which the powder particles are separated under the influence of a magnetic field produced within the closed receptacle and united to form magnetically anisotropic threads, chains or skeins hereinafter referred to as "magnetically anisotropic conglomerates." The latter, after removal from the closed receptacle, are compressed into a body which then is sintered to form a highly-coherent body.

These magnetically anisotropic threads, chains or skeins are unexpectedly quite resistant to the disorienting influence of external mechanical forces which are exerted on them when they are transferred to a die; in fact, formation of magnetically isotropic conglomerates virtually does not take place.

The invention is of particular importance for the manufacture of ceramic anisotropic magnets having as the constituent essential for the permanent magnetic properties

at least one material, in the form of hexagonal crystals, with a chemical composition according to the formula  $MO.6Fe_2O_3$ , where M is at least one of the metals Ba (barium), Sr (strontium) and Pb (lead). The proportions of the Weiss domains of the said crystals generally lie within the range of approximately 1 to 3 microns, so that for an average particle size under 1 micron, for example approximately 0.3 micron, by far most of the particles each are single Weiss domains. That is to say, these particles are micro-magnets magnetized spontaneously and up to the saturation, which have a strong tendency to conglomerate while forming the above-mentioned magnetically isotropic conglomerates. However, if it is possible to substantially prevent this conglomeration, a maximum magnetic orientation effect can actually be obtained just in this case. The present invention offers a means which is excellently suited to this purpose.

According to a particular embodiment of the invention, the permanent magnetic material from which the magnet body to be manufactured is constituted, is disintegrated and whirled to form a cloud of dust in a container which is closed with a cover on the inside of which the above-mentioned "magnetically anisotropic conglomerates," i.e. threads, chains or skeins deposit.

25 The magnetic field, under the influence of which the magnetically anisotropic threads, chains or skeins are formed, is usually produced by an electromagnet which is rendered operative after at least a part of the permanent magnetic material is disintegrated to an average particle size under 1 micron and is whirled to form a cloud of dust. Preferably, the electromagnet is provided in the cover of the container.

30 The invention will now be described with reference to a particular example which is illustrated only, and the accompanying drawing the sole figure of which shows an apparatus for carrying out the invention.

35 Finely-divided permanent magnet material 8, e.g. barium hexaferrite,  $BaO.6Fe_2O_3$ , initially ground in a ball mill, is placed in a metal container 1 provided with a metal cover 4 which hermetically seals the container. Cover 4 is provided with a neck 5 in which a soft iron magnet core 6 is provided which is wound with wire turns 7, the core and the wire turns together forming an electromagnet. Extending through the bottom of the container is a shaft 2 which supports a set of blades 3 for rotation.

40 After the apparatus has been switched on, the permanent magnetic powder is disintegrated by the metal bands, rotating at high speed, to an average particle size of approximately 0.5 micron, and whirled to form a cloud of dust. Two minutes later the electromagnet is switched on. In the neck of the cover the magnetically anisotropic threads, chains or skeins 9 of powder particles soon deposit in large numbers. After another two minutes grinding is discontinued, the cover is removed from the container, its lower side placed over a filling funnel, and the electromagnet switched off. The magnetically anisotropic chains are no longer attracted by the cover and fall into the filling funnel. From there the mass is transferred to a die, in which by means of an electromagnet a substantially homogeneous magnetic field is produced. The mass is then compressed in the magnetic field under a pressure of  $0.5 \text{ ton/cm}^2$ . The compressed body is removed from the die and sintered by heating it for 24 hours at a maximum temperature of  $1290^\circ \text{ C}$ . The resulting magnet body at room temperature has a  $(BH)_{\max}$  of  $3.8 \times 10^6$  gauss oersted and a magnetic anisotropy, expressed in the value of the quotient  $B_{r11}/B_{r1}$ , of 4.0 (where  $B_{r11}$  is the maximum remanence measured in a direction parallel to the principal direction of magnetization and  $B_{r1}$  the remanence measured in the direction at right angles to the di-

rection in which the maximum remanence  $B_r$  is measured).

While we have described the invention with reference to a particular apparatus and a particular material, it will be obvious to those skilled in the art that other forms of apparatus and other materials could be used equally well. For instance, instead of barium hexaferrite, other well-known magnetic materials such as magnetic alloys which can be formed into sintered bodies may be subjected to a similar treatment. Likewise, the material could be ground initially to the required fine state of subdivision and centrifuged by a conventional centrifuge, the magnetic field being applied from an external source.

Therefore, we wish it to be clearly understood that the foregoing example is illustrative only, the invention itself being limited only and defined by the appended claims.

We claim:

1. A method of manufacturing a magnetically anisotropic body comprising the steps, disintegrating a finely-divided magnetic material in a closed receptacle, whirling said material in said receptacle to form a dust cloud of said material, separating particles of said material in said dust cloud with a magnetic field which forms magnetically anisotropic conglomerates of said particles, removing said conglomerates from said receptacle, compressing the magnetically anisotropic conglomerates of said particles in the presence of a magnetic field into a body, and sintering said body to form the same into a highly coherent body.

2. A method of manufacturing a magnetically anisotropic body comprising the steps, disintegrating a finely-divided magnetic material having a composition consisting of  $MO \cdot 6Fe_2O_3$  where M is a metal selected from the group consisting of Ba, Sr and Pb in a closed receptacle, whirling said material in said receptacle to form a dust cloud of said material, separating particles of said material in said dust cloud with a magnetic field which forms magnetically anisotropic conglomerates of said particles, removing said conglomerates from said receptacle, compressing the magnetically anisotropic conglomerates of said particles in the presence of a magnetic field into a body, and sintering said body to form the same into a highly coherent body.

30

3. A method of manufacturing a magnetically anisotropic body comprising the steps, disintegrating a finely-divided magnetic material consisting essentially of  $BaO \cdot 6Fe_2O_3$  in a closed receptacle, whirling said material in said receptacle to form a dust cloud of said material, separating particles of said material in said dust cloud with a magnetic field which forms magnetically anisotropic conglomerates of said particles, removing said conglomerates from said receptacle, compressing the magnetically anisotropic conglomerates of said particles into a body in the presence of a magnetic field to form a magnetically anisotropic body, and sintering said body to form the same into a highly coherent body.
4. A method of manufacturing a magnetically anisotropic body comprising the steps, disintegrating a finely-divided magnetic material consisting essentially of  $BaO \cdot 6Fe_2O_3$  in a closed receptacle, whirling said material in said receptacle to form a dust cloud of said material, separating particles of said material in said dust cloud with a magnetic field which forms magnetically anisotropic conglomerates of said particles, removing said conglomerates from said receptacle, compressing the magnetically anisotropic conglomerates of said particles into a body in the presence of a magnetic field to form a magnetically anisotropic body, and sintering said body at a temperature of about  $1290^{\circ}C$ . for twenty-four hours to form the same into a highly coherent body.

#### References Cited

##### UNITED STATES PATENTS

|              |         |                |       |          |
|--------------|---------|----------------|-------|----------|
| 2,186,659    | 1/1940  | Vogt           | ----- | 29—155.6 |
| 2,384,215    | 9/1945  | Toulmin et al. | ----- | 29—420   |
| 2,856,273    | 10/1958 | Beeber et al.  | ----- | 23—288.3 |
| 35 2,974,887 | 3/1961  | Grandinetti    | ----- | 241—101  |
| 3,033,474    | 5/1962  | O'Toole        | ----- | 241—101  |
| 3,090,107    | 5/1963  | Minden et al.  | ----- | 29—155.6 |
| 3,189,667    | 6/1965  | Buttner et al. | ----- | 29—155.6 |

40 CHARLIE T. MOON, Primary Examiner.

C. E. HALL, J. W. BOCK, Assistant Examiners.